

1,512,961

Oct. 28, 1924.

E. H. WEIL

MANIFOLD

Original Filed Feb. 11, 1918



Inventor  
EDGAR H. WEIL

By Edward R. Alexander  
Attorney

## UNITED STATES PATENT OFFICE.

EDGAR H. WEIL, OF CLEVELAND, OHIO, ASSIGNOR TO THE VITREOUS ENAMELING COMPANY, OF CLEVELAND, OHIO, A CORPORATION OF OHIO.

## MANIFOLD.

Original application filed February 11, 1918, Serial No. 216,605. Divided and this application filed June 1, 1920. Serial No. 385,440.

To all whom it may concern:

Be it known that I, EDGAR H. WEIL, a citizen of the United States, residing at Cleveland, in the county of Cuyahoga and State of Ohio, have invented certain new and useful Improvements in and Relating to Manifolds, of which the following is a specification.

This invention relates to a manifold, more particularly a manifold for engines of the internal combustion type.

This application is a division of my application Ser. No. 216,605, filed Feb. 11, 1918.

In modern internal combustion engine and self propelled vehicle construction practice, it has been found advantageous, and in fact, essential to reduce, in one way or another, without sacrificing strength and durability, the weight of many of the parts and elements constituting the engine. With the increased cost of fuel and tires, this question has perhaps become foremost in the minds of the automobile manufacturer and engineer.

In solving this problem in connection with a manifold for internal combustion engines, serious conditions have to be met with respect to the high temperatures of the exhaust gases and chemical and atmospheric actions both of which are materially increased where accompanied by the heat of the exhaust gases.

The object of the invention is to provide a relatively light, durable manifold formed from sheet steel having its inner surface or both its inner and outer surfaces coated with a material which adequately protects it or them from the heat of the exhaust gases and from chemical action due to any causes whatever.

For the purpose of illustration, I have, in the accompanying drawing shown and herein described one form of device embodying my invention.

Referring to the drawing, Fig. 1 is an elevation of a manifold embodying my invention.

Figs. 2 and 3 are longitudinal and transverse sections, respectively, of the manifold.

In the drawing, 1 indicates as an entirety a manifold. In the manifold shown by way of example, the walls *a* thereof are shaped to provide a main section 1<sup>a</sup> and branches

1<sup>b</sup> adapting it for use in a Ford engine. 55 The manifold 1 is formed from sheet metal, preferably sheet steel, which not only insures a light-weight manifold but permits manufacture at relatively low cost.

B indicates a relatively thin coat of vitreous porcelain enamel uniformly applied to or upon the inner surfaces of the manifold section 1 and its branch members *a*; B' indicates a relatively thin coat of vitreous porcelain enamel uniformly applied to or 60 upon the outer surfaces thereof. As shown, the coats B, B', completely and uniformly cover the surfaces of the manifold to insure that no surfaces of the metal are exposed. The coat or coats B, B', serve to 65 adequately protect the metal walls *a* of the manifold so that it may be made from relatively thin material to reduce its weight and also from material that is relatively 70 cheap and easily worked, such as sheet iron 75 or steel.

I am aware of the fact that such material easily deteriorates on account of chemical action, especially where such action is accompanied with heat, and may be burned by 80 the extreme heat of the gases, but I have found that a manifold coated with vitreous porcelain enamel, especially when uniformly coated on both its inner and outer surfaces, is durable and capable of withstanding the 85 heat of the exhaust gases and chemical actions of all kinds. As the enameled surface of surfaces of the metal is or are entirely and uniformly coated or protected, it will readily be understood that no surfaces of the metal 90 are left exposed and accordingly no chemical action can take place even in the presence of the high temperatures of the exhaust gases. Accordingly, the manifold, although made from relatively thin material 95 (thereby effecting a material reduction in weight) and from material in which chemical action readily takes place, is so protected from the elements, the heat of the exhaust gases, as well as the chemical action incident to these gases, that it may be used as 100 an exhaust manifold for internal combustion engines with entirely satisfactory results under any and all conditions.

It may be noted that with a coating of 105 vitreous porcelain enamel on one or both walls of a relatively thin sheet metal manifold, the sheet metal is strengthened or stiff-

ened thereby, even though such coating be comparatively thin so that a relatively stiff construction is produced from relatively thin sheet metal. By taking advantage of 5 this property of enamel as well as its well-known protective properties, I am enabled to produce an extremely light manifold which will have great strength and rigidity and which will be durable because the metal 10 is protected from the attack and chemical action of the hot exhaust gases from the internal combustion engine.

So far as preventing burning of the metal on account of the high temperatures of the 15 exhaust gases is concerned, this result is accomplished by the coating B. To prevent chemical and atmospheric action on the outside of the manifold, as well as to give it a neat appearance, I prefer to provide the 20 coat B' in all instances.

To those skilled in the art, many modifications of and widely differing embodiments and applications of my invention will suggest themselves, without departing from the 25 spirit and scope thereof. My disclosures and descriptions herein are purely illustrative and are not intended to be in any sense limiting.

What I claim is:

30 1. A manifold for internal combustion engines and the like comprising an integral body of sheet metal having a relatively thin, substantially uniform coating of vitreous

enamel upon its inner and outer surfaces whereby a relatively light, stiff, protected 35 metal manifold is produced.

2. A manifold for internal combustion engines formed from relatively light sheet metal and having a substantially uniform coating of vitreous enamel upon its inner 40 and outer surfaces.

3. A manifold for internal combustion engines formed from relatively light sheet metal and having a relatively thin, substantially uniform coating of vitreous enamel 45 upon one of its surfaces, whereby a relatively light, stiff metal manifold is produced.

4. A manifold formed from sheet metal and having its interior walls coated with vitreous porcelain enamel. 50

5. A manifold formed from sheet metal and having its interior and exterior walls coated with vitreous porcelain enamel.

6. A manifold for an internal combustion engine formed from sheet steel and having 55 its inner surface coated with a relatively thin uniform coat of vitreous enamel.

7. A manifold for an internal combustion engine formed from sheet steel and having its inner and outer surfaces protected by relatively thin uniform coats of vitreous enamel. 60

In testimony whereof, I have hereunto signed my name.

EDGAR H. WEIL.